

# UNITED STATES PATENT OFFICE.

DMITRIE S. KONDRAIEFF, OF WILMINGTON, DELAWARE, ASSIGNOR OF ONE-HALF TO  
BERNARD EDELHERTZ, OF NEW YORK, N. Y.

## PROCESS OF MAKING SMOKELESS POWDERS.

1,212,770.

Specification of Letters Patent. Patented Jan. 16, 1917.

No Drawing.

Application filed November 16, 1916. Serial No. 131,668.

To all whom it may concern:

Be it known that I, DMITRIE S. KONDRAIEFF, a subject of Russia, residing at Wilmington, in the county of New Castle, State of Delaware, have invented certain new and useful Improvements in the Processes of Making Smokeless Powders; and I do hereby declare the following to be a full, clear, and exact description of the invention, such 10 as will enable others skilled in the art to which it appertains to make and use the same.

Up to the present time smokeless gun and rifle powders have been made from nitrocellulose which has been gelatinized. After 15 treating the cotton-wool or cellulose with nitric acid, it has been considered necessary to thoroughly wash the end products with water, so as to thoroughly remove any trace 20 of the free acids which would be undesirable and dangerous in the further treatment of the nitrocellulose. As a result the nitrocellulose is obtained in a wet condition. While it is in such wet condition the nitrocellulose is usually subjected to the well 25 known process of centrifuging after the nitrocellulose still contains a certain degree of moisture averaging from 25% to 30%.

It has heretofore been considered necessary 30 as an initial step, to subject the nitrocellulose, after centrifuging, to various processes of either thorough or partial drying or dehydration. The process of either thorough or partially drying or dehydrating the 35 nitrocellulose, after centrifuging, has been accomplished by various means and has been heretofore deemed necessary, in order to render the nitrocellulose soluble for the 40 purpose of bringing it into a condition required for the proper gelatinization of the nitrocellulose and ether for making an alcohol ether smokeless powder. Another commonly used method has been to treat the nitrocellulose with alcohol by percolation 45 with pressure. In all instances, these various processes of either thoroughly or partially drying the nitrocellulose, after centrifuging, or drying, or treating the nitrocellulose with alcohol by percolation with pressure, are expensive and take up a great deal 50 of time.

I have discovered that it is not necessary to remove any further part of the moisture from the nitrocellulose, after its centrifug-

ing, and that, in fact, the moisture remaining in the nitrocellulose, after such centrifuging, not only does not harm the degree of solubility, but, on the contrary, will greatly facilitate and improve it.

My new and improved process therefore, 60 consists in taking wet nitrocellulose and after removing from such nitrocellulose the usual amount of water, by means of centrifuging, and immediately without subjecting such nitrocellulose to any process of either 65 thorough or partial drying or dehydration, and without subjecting it to any process of drying with alcohol by percolation with pressure, adding to such wet or undried nitrocellulose simultaneously alcohol and ether in 70 the following proportions: To each 100 lbs. of nitrocellulose about 75 lbs. of alcohol and ether, one part alcohol and two parts ether. This admixture added as described, will bring about the condition required for the 75 proper gelatinization of the nitrocellulose and ether for the purpose of making an alcohol ether smokeless powder.

It is to be understood that the exact proportion of moisture in the wet or undried 80 nitrocellulose, after centrifuging, for the purpose of obtaining the most favorable results, may vary with a specific nitrocellulose used, as this is not at all times an absolutely uniform product, which variations 85 are well known to those skilled in the art. Similarly, therefore, changes may be made in the details of my invention, without departing from the spirit thereof.

### I. claim:

1. In the art of making smokeless gun and rifle powders, from nitrocellulose, that step which consists in adding alcohol and ether to the wet nitrocellulose, unsubjected to any other process of drying or dehydration except centrifuging, for the purpose of bringing about the condition required for the proper gelatinization necessary to produce an alcohol ether smokeless powder.

2. In the art of making smokeless gun 100 and rifle powders, from nitrocellulose, that step which consists in adding alcohol and ether to the wet nitrocellulose, after centrifuging, without subjecting such nitrocellulose to any other process of either thorough 105 or partial drying or dehydration, or to any process of drying with alcohol by percolation with pressure, for the purpose of bring-

ing about the condition required for the proper gelatinization necessary to produce an alcohol ether smokeless powder.

3. In the art of making smokeless gun and rifle powders, from nitrocellulose, that step which consists in adding simultaneously alcohol and ether to the wet nitrocellulose, immediately after centrifuging, without subjecting such nitrocellulose to any 10 other process of either thorough or partial drying or dehydration, or to any process of drying with alcohol by percolation with

pressure, for the purpose of bringing about the condition required for the proper gelatinization necessary to produce an alcohol 15 ether smokeless powder.

In testimony that I claim the foregoing as my invention, I have signed my name in presence of two subscribing witnesses.

DMITRIE S. KONDRATIEFF.

Witnesses:

BERNARD EDELIERTZ,  
EMANUEL LESVICK.